

## UNITED STATES PATENT OFFICE

2,593,496

## ADDITION AGENT AND MINERAL OIL LUBRICANT COMPOSITIONS CONTAINING THE SAME

Herschel G. Smith, Wallingford, and Troy L. Cantrell, Lansdowne, Pa., assignors to Gulf Oil Corporation, Pittsburgh, Pa., a corporation of Pennsylvania

No Drawing. Application February 4, 1948,  
Serial No. 6,344

25 Claims. (Cl. 252—46.6)

1

This invention relates to addition agents and mineral oil lubricant compositions containing the same and, more particularly, it is concerned with improvement agents which confer improved antioxidant, corrosion-inhibiting and pressure-carrying properties on mineral oil lubricants.

It is recognized in the art that mineral oil lubricants are readily oxidized under service conditions thereby reducing the service life of internal combustion engines and steam turbines. A concomitant effect is corrosion of bearing surfaces. These problems become particularly acute when a highly refined paraffinic base mineral oil is employed as the lubricant.

In the lubrication of internal combustion engines of all types, particularly when severe operating conditions are encountered, mineral lubricating oils frequently prove unsatisfactory because they tend to deposit varnish, gum and sludge on the engine surfaces, such as the cylinder walls, pistons and rings, and also to induce corrosion of bearing materials thereby causing failure of the engine. These problems have become increasingly serious because of the trend toward higher efficiency or higher power output per unit weight of engine, which results in conditions tending to accelerate the deteriorating influences on the mineral oil lubricant. The formation of so-called varnishes and sludges on engine surfaces is a result of oxidation effects on the lubricating oils. The presence of gums, varnishes and sludges is detrimental for many reasons. These substances tend to increase ring sticking and accelerate the formation of further deposits on piston surfaces and in fixed parts of the combustion chamber. The sludges formed in the crankcase of the engine increase the rate of corrosion of bearing surfaces, especially of bearing alloys of the types now in use.

In steam turbines, the corrosion problem is particularly acute because of the presence of water in the mineral oil lubricant and in addition to bearing corrosion, rusting may also be encountered.

It is an object of this invention, therefore, to prepare an improvement agent which will obviate the oxidation and corrosion difficulties encountered in the use of mineral oil lubricants.

It is a further object of this invention to provide improved mineral oil lubricant compositions which are stable in storage and use and in which oxidation and corrosion effects are materially inhibited.

2

It is also an object of this invention to provide mineral oil lubricant compositions which have excellent pressure-carrying properties.

In our copending application Serial No. 718,902, filed December 27, 1946, there is disclosed and claimed an addition agent for mineral oil lubricants which confers excellent antioxidant, corrosion-inhibiting and pressure-carrying properties on mineral oil lubricants. Such improvement agent is prepared by heating an essentially paraffinic base lubricating oil with aluminum chloride, removing aluminum chloride from the reaction product and reacting said product with phosphorus pentasulfide at an elevated temperature to incorporate phosphorus and sulfur therein.

In our copending application Serial No. 736,618, filed March 24, 1947, now U. S. Patent No. 2,456,336, there is disclosed and claimed an improvement agent for mineral oil lubricants which is prepared by heating an essentially paraffinic base lubricating oil with phosphorus pentasulfide in the presence of a surface active silica-containing solid catalyst. It is shown in that application that when phosphorus pentasulfide is reacted with an essentially paraffinic base lubricating oil in the presence of a surface active silica-containing solid catalyst, the prior aluminum chloride treatment of the lubricating oil as disclosed in our application Serial No. 718,902 may be omitted. It is also shown in our latter filed application that when the prior aluminum chloride treatment of the paraffinic base lubricating oil is combined with reaction of the aluminum chloride treated product with phosphorus pentasulfide in the presence of a surface active silica-containing catalyst, lighter colored products are obtained.

The objects of the present invention are accomplished by providing improvement agents for mineral oil lubricants by reacting an essentially paraffinic base lubricating oil or the aluminum chloride treated product thereof with phosphorus pentasulfide through the use of any of the methods disclosed in our copending applications Serial Nos. 718,902 and 736,618 and then reacting the resulting product with an ester having the formula:



50 wherein R and R<sub>1</sub> represent aliphatic hydrocarbon radicals, at least one of said radicals containing olefinic unsaturation, and the sum of the

carbon atoms of both R and R<sub>1</sub> being not less than 16. Such improvement agents, as well as the mineral oil lubricant compositions containing them, are believed to be novel and are considered parts of our invention.

The present invention may be regarded as an improvement over the inventions disclosed in our above-identified copending applications. While the addition agents disclosed therein confer excellent antioxidant, corrosion-inhibiting and pressure-carrying properties on mineral oil lubricants, they sometimes fail to pass the well known Copper Strip Test (Method 530.31, Federal Specification VV-L-791c, May 12, 1945, page 259) thus indicating the presence of elementary sulfur or the so-called "corrosive" sulfur. While we do not wish to be bound by any theory as to the exact nature of our phosphorus pentasulfide reaction products, it is our present belief that either elementary sulfur or incompletely bound sulfur or both are formed in the reaction. In accordance with the present invention, such elementary or incompletely bound sulfur is "neutralized" by combination with the unsaturated ester added to the phosphorus pentasulfide reaction product. In addition, the resulting products have enhanced pressure-carrying properties.

It is still necessary for the purposes of the present invention to employ an essentially paraffinic base lubricating oil as the initial material, because other hydrocarbon materials produce a black, sludge-like, difficultly soluble product regardless of whether the prior aluminum chloride treatment or reaction in the presence of a surface active silica-containing solid catalyst are employed. The reasons for the advantageous effects of the prior aluminum chloride treatment or of the surface active silica-containing solid catalyst on the reaction when an essentially paraffinic base lubricating oil is employed are not fully understood. However, the use of at least one of these methods is essential for the practice of our invention since, if the prior aluminum chloride treatment or the use of a surface active silica-containing catalyst is omitted, the advantageous results of our invention are not obtained. In order to obtain the results of our invention, therefore, it is necessary (1) to employ an essentially paraffinic base lubricating oil, and (2) to conduct the reaction of the oil with phosphorus pentasulfide only after aluminum chloride has been reacted with the oil and/or the reaction with phosphorus pentasulfide is conducted in the presence of a surface active silica-containing solid catalyst.

The essentially paraffinic base lubricating oil used as a starting material in accordance with our invention may be derived from any paraffinic crude, such as Pennsylvania, Mid-Continent, or other paraffinic base crudes. The lubricating oil is manufactured from such crudes in accordance with conventional methods and may be refined in accordance with methods known in the art. If it is desired to treat the essentially paraffinic base lubricating oil with aluminum chloride, such treatment is accomplished as described in our copending application, Serial No. 718,902. Briefly, such treatment comprises heating the essentially paraffinic base lubricating oil with from 1 to 20 per cent by weight of anhydrous aluminum chloride at a temperature of from 150° to 300° F. while the mixture is vigorously agitated. The time of treatment may vary in accordance with the amount of aluminum chloride used and the temperature of treatment, longer times being required with less aluminum chloride and lower

temperatures. In general, the treatment will be completed after four or five hours. After the treatment is completed, agitation is stopped and the sludge containing most of the aluminum chloride settles out from the main body of the oil and is drawn off. The supernatant body of the treated oil may contain further quantities of aluminum chloride finely dispersed therethrough, and in order to insure the removal of all aluminum chloride from the treated oil, agitating with an adsorbent clay followed by filtration may be employed. At the higher temperatures of treatment with aluminum chloride some conversion of the paraffinic base oil to lower boiling products may take place. Although such conversion is slight, the product may be topped if desired, that is, distilled to remove the lower boiling products overhead and to recover as a residue the bulk of the aluminum chloride treated oil having a minimum initial boiling point in the range 490° to 530° F.

The essentially paraffinic base lubricating oil treated with aluminum chloride as disclosed hereinabove may then be reacted with phosphorus pentasulfide. This may be accomplished either by reacting with phosphorus pentasulfide per se, as disclosed in our copending application Serial No. 718,902, or in the presence of a surface active silica-containing solid catalyst as disclosed in our copending application, Serial No. 736,618.

If it is desired to react the aluminum chloride treated oil with phosphorus pentasulfide per se, this reaction is accomplished by adding from 2 to 20 per cent by weight of P<sub>2</sub>S<sub>5</sub>, preferably 5 to 10 per cent, and heating with agitation at a minimum reaction temperature of 450° F. and a maximum reaction temperature below the temperature where cracking of the oil begins. Hydrogen sulfide is evolved and when the evolution of hydrogen sulfide has nearly ceased, the temperature of the reaction mixture may be increased within the maximum temperature disclosed above, say to about 500° F. for the completion of the reaction.

If desired, the aluminum chloride treated paraffinic base lubricating oil may be reacted with phosphorus pentasulfide in the presence of a surface active silica-containing catalyst; or, the prior aluminum chloride treatment may be omitted and the essentially paraffinic base lubricating oil may be reacted with phosphorus pentasulfide in the presence of a surface active silica-containing solid catalyst. The reaction of the essentially paraffinic base lubricating oil, whether or not pretreated with aluminum chloride, with phosphorus pentasulfide in the presence of a surface active silica-containing solid catalyst is accomplished by adding 2 to 20 per cent by weight of P<sub>2</sub>S<sub>5</sub>, preferably from 5 to 10 per cent, to the essentially paraffinic base lubricating oil and heating with agitation at a temperature in the range from 300° F. to a maximum temperature below the temperature where cracking of the oil, that is, pyrolytic decomposition of the oil, begins. Generally the minimum cracking temperature of the oil varies between 490° to 530° F., depending upon the particular oil used. The surface active silica-containing solid catalyst is employed in amounts of from 2 to 25 per cent by weight of the oil charged and preferably in an amount of 10 per cent by weight. Larger amounts than 10 per cent are ordinarily not necessary, but larger amounts will produce a product having a lighter color. During the course of the reaction hydrogen sulfide is evolved and the phosphorus and sulfur become incorporated in the oil. When

## 5

the evolution of hydrogen sulfide has nearly ceased, the temperature of the reaction mixture may be increased within the maximum temperature mentioned above, say to about 500° F., for completion of the reaction. The mixture may then be filtered to remove the catalyst, or the catalyst may be removed after further reaction of the product with an unsaturated ester as disclosed herein.

The surface active silica-containing solid catalysts may comprise activated clays, silica-alumina cracking catalyst and the like. Thus, activated clays, that is, natural clays such as bentonite, smectite, floridin, fuller's earth and the like which have been treated with acid, such as are described in U. S. Patent No. 1,898,165, for example, may be advantageously employed. Synthetic silica-alumina catalysts of the type used for the cracking of hydrocarbon oils, examples of which are described in U. S. Patent No. 2,078,945 and U. S. Patent No. 2,283,173, may also be employed. Activated silica gel is also suitable. As may be seen, the term "surface active silica-containing solid catalyst" comprises a wide variety of materials, the predominant characteristic of which is the presence of silica in a surface active, that is, activated form.

After reaction of the essentially paraffinic base lubricating oil with the phosphorus pentasulfide as disclosed hereinabove, the resulting reaction products are reacted, in accordance with the present invention, with an ester having the formula:



wherein R and R<sub>1</sub> represent aliphatic hydrocarbon radicals, at least one of said radicals containing olefinic unsaturation, and the sum of the carbon atoms of both R and R<sub>1</sub> being not less than 16. The reaction with the ester takes place at a temperature in the range 300° to 400° F., preferably about 350° F. The ester is ordinarily added in proportions ranging from 1.0 to 10 per cent by weight of the reaction mixture, sufficient to combine with free or "corrosive" sulfur in the phosphorus pentasulfide reaction product. When reacted under these conditions, we believe that the ester is linked to the phosphorus pentasulfide reaction product through a sulfur atom, and any free sulfur will also react with the ester.

Among the esters encompassed by the present invention and having the formula:



as defined hereinabove, there are included the following types:

(1) Those esters in which both R and R<sub>1</sub> have olefinic unsaturation. These include such esters as allyl oleate, decylene oleate, dodecylene oleate, pentadecylene oleate, oleyl oleate, and particularly sperm oil which provides an excellent source of this type of ester.

(2) These esters in which R has olefinic unsaturation, but R<sub>1</sub> is saturated. These include methyl oleate, isopropyl oleate, hexyl oleate, lauryl oleate, cetyl oleate and the like. In lieu of esters of oleic acid, esters of other olefinic mono-carboxylic fatty acids may be employed, such as esters of decenoic, undecenoic, linoleic and linolenic acids.

(3) Those esters in which R is saturated, but R<sub>1</sub> has olefinic unsaturation. These include allyl palmitate, decylene laurate, dodecylene caprylate and oleyl butyrate.

## 6

In selecting any ester of the above types, it should be borne in mind that the sum of the carbon atoms of R and R<sub>1</sub> must be not less than 16.

5 The following examples illustrate the preparation of our new improvement agents.

## Example I

10 Fifty-one parts by weight of an essentially paraffinic base lubricating oil (S.A.E. 30) which had been treated with aluminum chloride in accordance with our copending application Serial No. 718,902 were placed in a reaction vessel together with 5.6 parts by weight of phosphorus pentasulfide. The mixture was then agitated and heated to 450° F. for a period of 2 hours. The temperature was then gradually raised to 525° F. over a period of 4 hours and maintained at that point for 2 hours. The mixture was then cooled to 350° F. and 5.1 parts by weight of sperm oil were added. The mixture was held at this temperature for 4 hours and then cooled and diluted with an equal weight of a light lubricating oil, thereby forming a concentrate of the improvement agent. The product had the following properties:

|                         |      |
|-------------------------|------|
| Gravity, °API           | 24.0 |
| Viscosity, SUV, 100° F. | 520  |
| 30 Sulfur, per cent     | 1.94 |
| Phosphorus, per cent    | 1.68 |

## Example II

35 An essentially paraffinic base lubricating oil (S.A.E. 50) was pretreated with aluminum chloride as herein disclosed and reacted with 10 per cent by weight of phosphorus pentasulfide at 500° F. After completion of the reaction, 10 per cent by weight of the reaction mixture of sperm oil was added and the mixture agitated for 6 hours at 400° F. The product had the following properties:

|                         |      |
|-------------------------|------|
| Gravity, °API           | 23.4 |
| Viscosity, SUV, 100° F. | 1692 |
| Sulfur, per cent        | 4.5  |
| Phosphorus, per cent    | 1.6  |
| Neutralization No       | 0.04 |

## Example III

50 Five thousand four hundred parts by weight of an SAE 30 grade essentially paraffinic base lubricating oil were reacted with 600 parts by weight of phosphorus pentasulfide in the presence of 600 parts by weight of an activated clay catalyst at a temperature in the range 480° to 500° F. The reaction was completed after 6 hours. The mixture was then cooled to 350° F. and 600 parts by weight of sperm oil were added. The mixture was held at 350° F. for 2 hours and then filtered. The product had the following properties:

|                         |      |
|-------------------------|------|
| 65 Gravity, °API        | 22.6 |
| Viscosity, SUV, 210° F. | 78.7 |
| Color, NPA              | 6.5  |
| Sulfur, per cent        | 3.12 |
| Phosphorus, per cent    | 2.33 |
| 70 Neutralization No    | 13.9 |

The reaction products obtained in accordance with the preceding examples are excellent improvement agents for mineral oil lubricant compositions. They are light colored and readily

soluble in all types of mineral oils, that is paraffinic, naphthenic or mixed base mineral oils and, as a matter of fact, can be blended with mineral oils in proportions as high as 50 per cent by weight or higher. This excellent solubility of our new improvement agents enables the preparation of concentrated solutions, which may then be diluted down to the proportion desired in the final mineral oil lubricant composition. As stated, our new improvement agents confer excellent pressure-carrying, anti-oxidant and corrosion-inhibiting properties on the mineral lubricating oils with which they are incorporated. For these purposes, our new improvement agents are generally added to mineral oils in minor amounts, say from 0.1 to 20 per cent by weight of mineral oil, sufficient to confer improved pressure-carrying, anti-oxidant and corrosion-inhibiting properties on the mineral lubricating oils with which they are incorporated. When our new improvement agents are to be used for their anti-oxidant and corrosion-inhibiting effects, small proportions as low as 0.1 per cent by weight are sufficient to effect the improvement. When extreme pressure properties are to be conferred on a lubricating oil, higher proportions, as high as 20 per cent may conveniently be used. Lubricating oils containing our new improvement agents successfully pass the Copper Strip Test.

The following examples illustrate the use of our new improvement agents to obtain improved mineral oil lubricant compositions.

8 properties of the improved lubricant and the base lubricant follows:

|                                                         | Base Lubricant | Improved Lubricant |
|---------------------------------------------------------|----------------|--------------------|
| Gravity: ° API                                          | 28.2           | 28.3               |
| Viscosity, SUV:                                         |                |                    |
| 100° F.                                                 | 554            | 558                |
| 210° F.                                                 | 67.5           | 67.8               |
| Viscosity Index                                         | 101            | 102                |
| Color, N.P.A.                                           | 4.5            | 4.5                |
| Sulfur: Per Cent                                        | 0.18           | 0.19               |
| Phosphorus: Per Cent                                    | nil            | 0.03               |
| Neutralization No.                                      |                | 0.06               |
| Oxidation and Bearing Corrosion Test, Method 257, Gulf: |                |                    |
| Duration of Test: Hrs.                                  | 48             | 48                 |
| Oil Bath Temperature: ° F.                              | 347            | 347                |
| Air Rate: cc./Hr.                                       | 2,000          | 2,000              |
| Quantity of Oil: cc.                                    | 300            | 300                |
| Bearing Type                                            | Cd-Ag          | Cu-Pb              |
| Wt. Change: Grams                                       | -0.0989        | -0.1488            |
| Wt. Change: Per Cent                                    | -0.51          | -0.74              |
| Copper Strip Test                                       | Passes         | Passes             |

20

#### Example VI

In order to determine the improvement in pressure carrying properties obtained by using the addition agent of the present invention, additives 25 prepared in accordance with the disclosures of Serial No. 718,902, Serial No. 736,618 and in accordance with the present invention were blended 30 in a motor oil, and the lubricants were subjected to the well known Falex Wear Test. In each instance, 15 parts by weight of the addition agent were added to 85 parts by weight of a highly refined motor oil. The un compounded oil is included for purposes of comparison.

|                                                  | Uncompounded Lubricant | Lubricant of S. N. 718,902 | Lubricant of S. N. 736,618 | Lubricant of Present Invention |
|--------------------------------------------------|------------------------|----------------------------|----------------------------|--------------------------------|
| Gravity: ° API                                   | 29.3                   | 28.9                       | 28.8                       | 28.7                           |
| Viscosity, SUV: 100° F.                          | 246                    | 244                        | 245                        | 241                            |
| Color, N.P.A.                                    | 1.75                   | 1.75                       | 1.75                       | 1.75                           |
| Copper Strip Test                                | Passes                 | Tarnished                  | Tarnished                  | Passes                         |
| Falex Wear Test, 1,000 Lb., Gauge Load, 15 min.: |                        |                            |                            |                                |
| Wear: No. of Teeth                               | fails                  | 0                          | 0                          | 0                              |
| Gauge Load at Seizure: Lb.                       |                        | 1,750                      | 1,750                      | 2,000+                         |

#### Example IV

An improved motor oil was prepared by blending 0.3 per cent by weight of the additive of Example II with 99.7 per cent by weight of a highly refined motor oil. A comparison of the properties of the improved lubricant and the base lubricant follows:

|                                                         | Unimproved Lubricant | Improved Lubricant |
|---------------------------------------------------------|----------------------|--------------------|
| Gravity: ° API                                          | 29.2                 | 29.2               |
| Viscosity, SUV 100° F.                                  | 524                  | 526                |
| Color, N.P.A.                                           | 1.75                 | 1.75               |
| Oxidation and Bearing Corrosion Test, Method 257, Gulf: |                      |                    |
| Duration of Test: Hrs.                                  | 48                   | 48                 |
| Oil Bath Temperature: ° F.                              | 347                  | 347                |
| Air Rate: cc./Hr.                                       | 2,000                | 2,000              |
| Quantity of Oil: cc.                                    | 300                  | 300                |
| Bearing Type                                            | Cd-Ag                | Cu-Pb              |
| Wt. Change: Grams                                       | -0.500               | -0.250             |
| Wt. Change: Per Cent                                    | -0.25                | -0.06              |
| Copper Strip Test                                       | Passes               | Passes             |

#### Example V

An improved motor oil was prepared by blending 1 per cent by weight of the additive of Example III with 99 per cent by weight of a refined paraffinic base motor oil. A comparison of the

50 The "Oxidation and Bearing Corrosion Test, Method 257 Gulf" referred to in the foregoing examples is conducted as follows: An alloy bearing shell of certain commonly used standard dimensions is submerged in 300 cc. of the oil or oil composition to be tested in a 400 cc. Pyrex beaker and heated in a thermostatic oil bath to 370° F. Air is then bubbled through the oil in contact with the bearing shell at a rate of 2000 cc. per hour. 55 At the end of 48 hours the loss of weight and condition of the bearing shell are determined, the bearing shell being washed free of oil and dried before weighing. When determining the effectiveness of various improvement agents, the usual procedure is to run a blank test simultaneously with the oil composition being tested, employing for that purpose a sample of the untreated oil. In this test it is advantageous to employ commercial bearing shells. These shells 60 comprise a suitable metal backing faced with the alloy bearing metal. In this way the actual bearing face is subjected to severe deterioration conditions. By comparison of the results of such tests with actual service tests, we have found them to be in substantial agreement as to suitability of particular lubricants.

As shown in the above examples, the addition 65 of our new improvement agents to mineral oil lubricant compositions confers excellent pressure-carrying, anti-oxidant and corrosion-in-

hibiting properties. At the same time the compositions so obtained are stable in storage and use and have a color which is substantially unaffected by the addition of the improvement agent. The lubricants obtained pass the Copper Strip Test and show enhanced pressure-carrying properties over the lubricants of our copending applications.

While we have shown in the examples the preparation of compounded lubricating oils, our invention is not limited thereto but comprises all mineral oil lubricant compositions containing our new improvement agents, such as greases and the like. Furthermore, conventional addition agents such as viscosity index improvers, pour point depressants and the like may be added without departing from the spirit of the invention.

We claim:

1. The process of preparing an improvement agent for mineral oil lubricants which comprises heating an essentially paraffinic base lubricating oil with anhydrous aluminum chloride at a temperature of from 150° to 300° F., removing aluminum chloride from the reaction product, reacting said product with phosphorus pentasulfide at a temperature of from 450° F. to a maximum temperature below the minimum cracking temperature of said product to incorporate phosphorus and sulfur therein, and then further reacting the resulting product at a temperature of from 300° to 400° F. with an ester having the formula:



wherein R and R<sub>1</sub> represent aliphatic hydrocarbon radicals, at least one of said radicals containing olefinic unsaturation, and the sum of the carbon atoms of both R and R<sub>1</sub>, being not less than 16.

2. The process of claim 1, wherein the aluminum chloride is employed in an amount of from 1 to 20 per cent by weight, the phosphorus pentasulfide is employed in an amount of from 2 to 20 per cent by weight, and the ester is employed in an amount of from 1 to 10 per cent by weight, sufficient to combine with free or "corrosive" sulfur in the phosphorus pentasulfide reaction product.

3. The process of claim 2, wherein the ester is sperm oil.

4. The process of claim 2, wherein the product is dissolved in a mineral lubricating oil.

5. The process of preparing an improvement agent for mineral oil lubricants which comprises heating an essentially paraffinic base lubricating oil with phosphorus pentasulfide in the presence of a surface active silica-containing solid catalyst at a temperature of from 300° F. to a maximum temperature below the minimum cracking temperature of said lubricating oil to incorporate phosphorus and sulfur therein, and then further reacting the resulting product at a temperature of from 300° to 400° F. with an ester having the formula:



wherein R and R<sub>1</sub> represent aliphatic hydrocarbon radicals, at least one of said radicals containing olefinic unsaturation, the sum of the carbon atoms of both R and R<sub>1</sub> being not less than 16, and recovering the reaction product.

6. The process of claim 5, wherein the phos-

phorus pentasulfide is employed in an amount of from 2 to 20 per cent by weight, the catalyst is employed in an amount of from 2 to 25 per cent by weight and the ester is employed in an amount of from 1 to 10 per cent by weight, sufficient to combine with free or "corrosive" sulfur in the phosphorus pentasulfide reaction product.

7. The process of claim 6, wherein the ester is sperm oil.

8. The process of preparing an improvement agent for mineral oil lubricants which comprises heating an essentially paraffinic base lubricating oil with from 1 to 20 per cent by weight of anhydrous aluminum chloride at a temperature of from 150° to 300° F., removing aluminum chloride from the reaction product, heating said product with from 2 to 20 per cent by weight of phosphorus pentasulfide in the presence of from 2 to 25 per cent by weight of a surface active silica-containing solid catalyst at a temperature of from 300° F. to a maximum temperature below the minimum cracking temperature of the aluminum chloride treated oil to incorporate phosphorus and sulfur therein, and then further reacting the resulting product at a temperature of from 300° to 400° F. with an ester having the formula:



wherein R and R<sub>1</sub> represent aliphatic hydrocarbon radicals, at least one of said radicals containing olefinic unsaturation, the sum of the carbon atoms of both R and R<sub>1</sub> being not less than 16, and recovering the reaction product.

9. The process of claim 8, wherein the ester is sperm oil and is employed in an amount of from 1 to 10 per cent by weight, sufficient to combine with free or "corrosive" sulfur in the phosphorus pentasulfide reaction product.

10. The product obtained by the process of claim 1.

11. The product obtained by the process of claim 2.

12. The product obtained by the process of claim 4.

13. The product obtained by the process of claim 5.

14. The product obtained by the process of claim 8.

15. A lubricant composition comprising a major amount of a mineral lubricating oil and a minor amount, sufficient to confer improved bearing corrosion-inhibiting properties on the composition of the product obtained by the process of claim 1.

16. A lubricant composition comprising a major amount of a mineral lubricating oil and a minor amount, from 0.1 to 20 per cent by weight, of the product obtained by the process of claim 2.

17. A lubricant composition comprising a major amount of a mineral lubricating oil and a minor amount, sufficient to confer improved bearing corrosion-inhibiting properties on the composition, of the product obtained by the process of claim 5.

18. A lubricant composition comprising a major amount of a mineral lubricating oil and a minor amount, from 0.1 to 20 per cent by weight, of the product obtained by the process of claim 6.

19. A lubricant composition comprising a major amount of a mineral lubricating oil and a minor amount, sufficient to confer improved

11

bearing corrosion-inhibiting properties on the composition, of the product obtained by the process of claim 8.

20. The product obtained by the process of claim 3.

21. The product obtained by the process of claim 7.

22. The product obtained by the process of claim 9.

23. A lubricant composition comprising a major amount of a mineral lubricating oil and a minor amount, from 0.1 to 20 per cent by weight, of the product obtained by the process of claim 3. 10

24. A lubricant composition comprising a major amount of a mineral lubricating oil and a minor amount, from 0.1 to 20 per cent by weight, of the product obtained by the process of claim 7. 15

12

25. A lubricant composition comprising a major amount of a mineral lubricating oil and a minor amount, from 0.1 to 20 per cent by weight, of the product obtained by the process of claim 9.

HERSCHEL G. SMITH.  
TROY L. CANTRELL.

## REFERENCES CITED

The following references are of record in the file of this patent:

## UNITED STATES PATENTS

| Number    | Name   | Date         |
|-----------|--------|--------------|
| 2,179,065 | Smith  | Nov. 7, 1939 |
| 2,179,067 | Smith  | Nov. 7, 1939 |
| 2,405,482 | Zimmer | Aug. 6, 1946 |